

# United States Patent Office.

THOMAS J. BARRON, OF BROOKLYN, NEW YORK.

Letters Patent No. 60,823, dated January 1, 1867.

## IMPROVED PROCESS FOR CONVERTING IRON INTO STEEL.

The Schedule referred to in these Letters Patent and making part of the same.

TO ALL WHOM IT MAY CONCERN:

Be it known that I, THOMAS J. BARRON, of Brooklyn, in the county of Kings, and State of New York, have invented a new and improved Method or Process of Converting Iron into Steel; and I do hereby declare that the following is a full, clear, and exact description thereof, and of its mode or manner of operation.

My invention or discovery consists in converting iron into steel, after the metal is formed or fashioned into any shape desired or required, and more or less deeply, as found useful or necessary, by the application of certain gases brought in contact with the metal while hot, and acting in combination with any suitable apparatus for heating such metal. The gases used by me for such purpose of converting iron into steel are carburetted hydrogen in combination with nitrogen or cyanogen separately or together, or carburetted hydrogen with nitrogen and carbonic oxide. Ammoniacal gas and chlorine may also be used in the place of or mixed with the nitrogen.

The manner of applying these gases and carrying out my invention is substantially as follows: I construct a furnace to contain one or more ovens, muffles, or retorts, of such form as to be adapted to receive the iron which it is desired to convert either partially or wholly into steel. Such retorts are to be brought to a bright red or white heat according to the character of the steel to be produced, when the iron is placed into them and the retort closed. Into such retorts there is then forced or caused to enter, in immediate contact with the iron or metal, a mixture of carburetted hydrogen and nitrogen or cyanogen gas, or of carburetted hydrogen and nitrogen acid, carbonic oxide gas, and either with or without gases derived from the compounds of ammonia. The carburetted hydrogen may be prepared in a separate retort in the usual manner, or may be generated in the retort containing the metal to be steeled, by slowly admitting into such retort either liquid hydro-carbons, solid hydro-carbons, or nitrogenized or other fats, which will be decomposed by the heat of the retort and converted into gas. The nitrogen is prepared in the usual manner and is then forced into the retort in connection with the carburetted hydrogen. A proportion of from one-sixth to one-quarter of nitrogen gas to five-sixths or three-quarters of carburetted hydrogen, will be found sufficient in ordinary cases to produce the result desired; but a larger proportion of nitrogen may be used, provided it is not so great as to drive the hydro-carbon from the surface of the metal, the surplus of the gases not taken up by the iron producing no injurious effect, except perhaps a cooling effect upon the heat of the retort, and passing out of the muffle. Cyanogen gas, which is composed of nitrogen and carbon, may be used in place of pure nitrogen, but in such case a little greater proportion of cyanogen than of nitrogen should be used or mixed with the carburetted hydrogen. The gases formed by the decomposition of the muriate or other salts of ammonia, or of any substance that will produce such gases, may also be used in place of the nitrogen or in connection with it; the latter I deem the most preferable form of use. A compound or mixed gas composed of nitrogen and carbonic oxide, with a small proportion of cyanogen and produced by passing atmospheric air through an air-tight retort, filled with charcoal, coke, or other fuel, and heated to ignition, may also be used in combination or connection with the carburetted hydrogen, and from the nitrogen and carbon contained in it, will be equally efficacious in producing the result mentioned. From the facility and cheapness with which such mixed gas is produced, I generally make use of it. Articles, which it is desired to coat with or convert into steel, are allowed to remain in the bath of gases a longer or shorter time according to the depth of the steel surface required or desired, and the degree of heat to which they are subjected in the retort. With a low degree of heat, a longer time is required to steel the metal to a given depth, and the greater the heat, the quicker the action of the gases, and the higher the steel. The time occupied in the process varies from a few seconds to a number of hours, five or six or more in some cases, according to the depth to which it is desired to steel the metal, and the character, and size, and thickness of the iron, and the heat of the furnace. I have converted iron one-sixteenth of an inch thick into good steel in three minutes, and half an inch thick by two inches wide, in one and a half hours. If the heat is high enough, iron will be converted into steel an eighth of an inch deep, in from five to ten minutes, and in a much less time when the metal is near a welding heat; but with such extreme heat, the metal becomes coarse and requires reworking. What will be a sufficient time in any case and under different circumstances, can be easily determined by the operator by one or two preliminary trials.

When the iron to be coated with or converted into steel is impure, chlorine gas should be admitted into the retort previous to the admission of the carburetted hydrogen and other gases, and should remain in contact with the metal a few minutes or longer time, according to the quality of the iron. Such gas has the effect to

60823

carry off or take up any impurities, as they are volatilized, which may have been contained in the metal. Such gas may be prepared and forced into the retort, or generated therein, as found most convenient. When the iron is pure, the use of the chlorine gas may be dispensed with. When the metal has been sufficiently acted on by the gases, in the hottest part of the retort, it may be removed to the end or cooler part of the retort, or to another retort connecting therewith and extending beyond the heat of the fire, and there retained in the bath of gases until it is sufficiently cool to prevent oxidation when it comes in contact with the atmosphere. This manipulation or removal is made when the metal or articles steeled do not require hardening. When any such articles require hardening the retort connects with or opens into the hardening bath, into which the articles are dropped without exposure to the atmosphere. When the retort cannot be connected with the hardening bath, a jet of the gases should be played upon the metal or articles as they are removed from the retort to the hardening bath, so as to form an atmosphere of gas around them to prevent oxidation. This shielding of the articles from contact with the atmosphere in passing from the retort to the hardening bath, prevents oxidation or discoloration of the surface, and is especially desirable and useful when the article has been polished or finished before being steeled, and it is desired to preserve perfect the finished or polished surface. The retorts containing the metal or articles to be steeled, are ventilated so as to allow the gases to escape therefrom; and fresh gas to enter or be generated therein, or a discharge-pipe may be connected therewith which will conduct the gases passing out of the retort into the fire, where they can be burned as fuel.

What I claim as my invention, and desire to secure by Letters Patent, is—

1. The use and application, for converting iron into steel, of the compound gas, composed of carburetted hydrogen with nitrogen and cyanogen, or with nitrogen and carbonic oxide, and either with or without ammoniacal and chlorine gases, applied substantially as described.
2. The use, in combination with the process of converting iron into steel by the application of such gases, of chlorine gas, preliminary to such process, for the purpose and in cases as set forth.
3. Protecting the metal, after it has been steeled or converted into steel, and when the same is to be hardened while being transferred to the hardening bath from contact with the atmosphere, for the purposes set forth.

THOS. J. BARRON.

Witnesses:

S. D. LAW,  
W. R. RICE.